# EUROPEAN PATENT SPECIFICATION

(11) **EP 1 373 654 B1**
(45) Date of publication and mention of the grant of the patent: **26.07.2006**
(21) Application number: 02718305.2
(22) Date of filing: 22.03.2002
(51) Int. Cl.: E04C 5/01

(54) **PROCESS FOR MANUFACTURING CORROSION RESISTANT METAL PRODUCTS**
VERFAHREN ZUR HERSTELLUNG VON KORROSIONSBESTÄNDIGEN METALLKÖRPERN
PROCEDE DE FABRICATION DE PRODUITS METALLIQUES RESISTANT A LA CORROSION

(30) Priority: 23.03.2001 GB 0107315
(43) Date of publication of application: 02.01.2004
(73) Proprietor: Hardy, Harmon Sidney, Dallas, TX 75220 (US); Cacace, Antonino Giorgio, Swansea, West Glamorgan SA3 3BU (GB)
(72) Inventor: CACACE, Antonino, Giorgio, Swansea, West Glamorgan SA 33BU (GB)
(74) Representative: Jones, Graham Henry
(86) International application number: PCT/GB2002/001402
(87) International publication number: WO 2002/077386

(56) References cited:
- EP-A- 0 059 070
- GB-A- 2 166 830
- US-A- 3 582 457
- US-A- 5 263 291
- US-A- 5 770 286

## Description

### FIELD OF THE INVENTION

This invention relates to a process for the manufacture of corrosion resistant metal products and to products produced from the process. The invention has particular but not necessarily exclusive application to products comprising a core formed from mild steel and having a stainless steel cladding. The term 'clad products' will be used herein to refer to such products. The present invention was conceived in the course of manufacturing such products in which the core is formed from recycled mild steel swarf but is not necessarily limited thereto. For example, the invention may also be applicable to products comprising a core formed from solid steel, powdered iron ore and even from other metals and metalliferous ores in which the problems identified herein are encountered.

Examples of such products, and processes for producing them, are described in the applicant's patent application #PCT/GB00/02894 and the several earlier patents referred to therein, the disclosures of all of which are incorporated herein by reference. It is therefore not considered necessary to describe these products and processes in detail here.

The term "engineering steel" is intended to describe those low alloy steels that are commonly subjected to machining operations including mild steel (a term that itself includes carbon steel), forging steel and axle or shaft steel all of which contain significant amounts of carbon.

For brevity and where convenient, 'stainless steel' will be referred to herein as 'ss'.

### BACKGROUND OF THE INVENTION

The background of the present invention is set out in detail in the specification of international patent application #PCT/GB94/00091. In the process described in that application, a billet comprised of an ss-jacket filled with briquettes of mild steel swarf is heated and worked into a finished product having the desirable properties and low cost of mild steel but that has an ss-cladding for substantially increased corrosion resistance.

In principle, the process is suitable for many traditional long products produced by conventional steel rolling techniques including plain and ribbed reinforcing bars ("rebars") for concrete constructions, round bars, flat bars, angle bars and channel bars.

There is a market for a rebar having a 75-100 year life under severely corrosive conditions. However, the core of an ss-clad rebar is exposed when it is cut. Studies have shown that, if left exposed, these cut ends could reduce the life of the concrete structure.

The techniques used to date to seal the bar ends include arc welding the ends with ss-wire (e.g by the MIG or TIG process) and welding ss-end caps or -discs onto the bar ends. A major disadvantage of these is the cost and the availability of skilled personnel, especially if on site welding of the cut ends has to be effected. A double ss-weld layer procedure is required. Typically a single end is welded in 5-10 minutes. At a welder's rate of £10/hr and the cost of ss-welding wire at £0.75/end, the total cost/end = £2.0.

The ends could be welded robotically. However, the cost of a robotic welder is of the order of £100 000 and that of the welding wire would remain £0.75/end.

Due to the lengths of typical rebars, the welds are usually effected in the horizontal position. In combination with the thin ss-cladding this makes it difficult to effect a perfect weld. Currently 30% of all ends have to be rewelded due to pin holes. These are clearly evident once a bar has been pickled.

In another sealing technique, heat-shrinking plastics caps are mounted on the ends. Such caps do not form a water-tight seal and they are prone to be damaged or dislodged in a building site environment. A study has been carried out on a 12-year old concrete motorway in New Jersey (USA) constructed with ss-clad rebars with heat-shrunk plastic caps at the ends. The only corrosion evident in the rebars was inside the end-caps where the carbon steel core had corroded.

Such technique is known through EP-A-059070, the end of a reinforcing bar being first sealed with a resin.

The applicant has made attempts to seal the bar ends by metal spraying. Metal spraying tends to be porous and has a brittle surface adherence. Porosity would lead to corrosion through the pores and therefore be ineffective. Furthermore metal sprayed ends would be prone to handling and on site damage.

Mild steel rebars have commonly been coated with an adhesive such as epoxy. The major weakness of such bars perceived by the market is that the epoxy coating is prone to sustaining damage during handling. Obviously the ends of ss-clad rebars would be equally prone to such damage, and this would therefore be perceived as a weakness by potential users.

### SUMMARY OF THE PRESENT INVENTION

In one aspect of the invention, there is provided a method of sealing a cut end of an elongate product comprising a core of corrosion susceptible metal and a cladding of corrosion resistant metal bonded to an axially extending outer face of the core, the method being defined by appended claim 1.

It will be clear to the skilled addressee that, in this specification and the claims, the term "corrosion susceptible metal" means a metal that is liable to corrosion in the conditions of service in which the product is intended to be used and is clad with a cladding of metal that is less susceptible to corrosion in those conditions of service than the metal of which the core is composed. Similarly, it will be clear that the term "corrosion resistant metal" has the inverse meaning.

Advantageously, according to the invention, any space between the cut end and the capping element is filled by sealant.

In one form of the invention, liquid sealant is inserted in the capping element before the capping element is mounted over the cut end of the product. This form of sealant advantageously take the form of a suitable resin such as polyurethane. The volume of the liquid sealant so provided advantageously exceeds the volume of the space between the cut end and the capping element after the capping element is mounted over the cut end so that, according to the invention, the cut end of the product displaces some of the liquid sealant from the capping element when the capping element is mounted over the cut end.

One advantage of using a resinous sealant is that the sealant cures to become non-fluent. Another advantage is that many such sealants are able to form a stable bond to both the cladding and the capping element.

In one form of the invention, the capping element is deformed after it is mounted over the cut end of the product to cause the volume of any space enclosed by the capping element to be reduced. This helps to eliminate voids in the space between the cut end and the capping.

Again in one form of the invention, sealant in a non-liquid state is present in the capping element when the capping element is mounted over the cut end of the product, the seal being created by steps that include causing the sealant to become liquid so that it flows between the skirt and the axially extending portion of the cladding.

In one form of the invention, the sealant is caused to become liquid by steps that include applying heat to cause the sealant to melt so that it flows between the skirt and the axially extending portion of the cladding, and subsequently allowing the sealant to resolidify.

Advantageously, according to the invention the sealant is metallic. A suitable solder or brazing alloy may be used for such a sealant.

In one form of the invention, the heat is applied by an induction heating apparatus.

In an alternative form of the invention, the skirt is caused to be in sealing contact with the cladding by at least one process selected from the group comprising crimping, swaging, forging or welding.

In one form of the invention, the capping element is of corrosion resistant metal, advantageously stainless steel.

The scope of the invention extends to products formed by the methods claimed herein.

### BRIEF DESCRIPTION OF THE DRAWINGS

Various embodiments of the invention are now discussed with reference to the accompanying drawings in which:
- Figure 1 is a side view, partly in section, of a ribbed rebar with capping elements positioned adjacent its ends;
- Figure 2 is a similar view of the rebar with the capping elements mounted over its ends;
- Figure 3 is a schematic view showing the layout of a set of crimping dies disposed in an open position about a capping element;
- Figure 4 is a similar view of the crimping dies in a closed position;
- Figure 5 is a side view of an ss-clad round bar or flat bar with capping elements mounted on its ends;
- Figure 6 is a schematic view of an apparatus used to apply end caps containing metallic sealant to the ends of rebars;

### DETAILED DESCRIPTION OF EMBODIMENTS OF THE INVENTION

Referring to Figure 1, a ribbed rebar 10 comprises a core 12 to which ss-cladding 14 is bonded. The ribs are shown at 16. The core is of mild steel or any other suitable grade of engineering steel. The cladding is of ASTM A316, A304 or any other suitable grade of stainless steel. In the present case, the rebar is produced by the process described in patent application #PCT/GB00/02894 and the earlier patents referred to therein. However, these are not essential conditions and, in principle, the invention may be applied to rebar and any other product of the type referred to herein produced by any other process and comprising a cladding of corrosion resistant metal bonded to a core of corrosion susceptible metal.

For the sake of illustration, the rebar 10 as shown is foreshortened. In practice the rebar will be much longer and will be cut to its designed length from parent stock of substantially greater length. At the cut end 13, a portion 18 of the core 12 is exposed at each end face. SS-clad bar of this kind is best cut to length by an abrasive cutter or other means that produce end faces that are square to the longitudinal axis of the bar. The cut ends are also desirably free of burrs and flashings. However, these goals are difficult to achieve economically or practically, especially where the cut is made on site. The method of the invention is nevertheless well suited to sealing the cut ends of clad products in such circumstances.

Capping elements 20 (hereinafter referred to simply as 'caps') are mounted over each cut bar end for this purpose. Each cap is cup shaped, having a circular base 22 integrally joined to a cylindrical skirt 24. In one embodiment, the cap is advantageously produced by deep drawing a disc stamped from a sheet of stainless steel of the same grade as the cladding. The cap may alternatively be of other suitable corrosion resistant metal, including another grade of stainless steel, that is compatible with whatever material the cladding is composed, particularly having regard to the avoidance of galvanic corrosion between the two metals when the rebar is in use.

In the example shown in Figures 1 and 2, a predetermined quantity of liquid resinous sealant, indicated schematically at 26, is inserted in the cap prior to mounting the cap on the bar end. Enough sealant should be inserted to ensure that, when the cap is mounted over the bar end, all of the space enclosed by the cap and not taken up by the bar end should be occupied by sealant. For this reason it will be necessary to insert an excess of sealant so that some of it is squeezed out by the bar end by the time it has been fully inserted into the skirt. A quantity of sealant equal to about 25% of the volume of the interior of the cap should be sufficient where the bar ends are reasonably square. More sealant, perhaps up to 50% of the same volume, may be required when the ends are cut at an angle or are jagged.

It is necessary that the skirt 24 must overlie the cladding completely when the bar end is fully inserted into the cap as shown at the left hand end of Figure 1. The depth of the skirt must be chosen accordingly. In this position, the skirt 24 is crimped or swaged against the cladding as shown in Figure 2, locking the two together and forming a seal that prevents the sealant when it is still liquid, from flowing out of the cap under gravity.

The term "crimping" refers to a process in which the skirt is squeezed tightly against the cladding without substantially deforming the cladding. On the other hand, in a "swaging" process, the applied force is sufficient to deform the cladding and perhaps more securely locking the cap on the bar. The term 'swaging' will hereinafter be used to cover both. In the swaging operation the skirt 24 is deformed inwardly. This tends also to cause some of the liquid sealant to be squeezed out. However, in the same process, the base 22 may become domed as shown at 22' in Figure 2. This may cause a void, indicated schematically as 30, between the cap and the bar end. Unless removed, the void may lead to corrosion of the exposed portion 18 of the core or crevice corrosion of the stainless steel. Voids can be removed by deforming the domed portion 22' of the base inwardly while the sealant is still liquid. This can be achieved simply by striking the domed portion with the rounded head of a hammer. This is an important consideration when, as often happens, the rebar has been cut on site. The domed portion is thus at least partly flattened as shown schematically at 22" or even domed inwardly, eliminating the void.

In due course the sealant cures, adhering to the surfaces of the cap and the bar end with which it is in contact and becoming non-fluent in the process. The sealant prevents corrosion of the exposed portion 18 of the core and the cap serves to protect the sealant and very effectively prolong it's life.

The sealant can be selected with regard to its suitability in the environment in which the end product is used. In the present instance, where the end product is a rebar for use in a concrete construction, the sealant is usefully a high quality polyurethane having good adhesive properties and a long life. Suitable proprietary products, used for used for sealing roofs, are available under the Nurethane and Nuflex trade names and have a guaranteed life of 30 years when used for that purpose. Other organic materials, including certain flexible epoxies, may also be suitable. The sealant must be resistant to alkaline attack since freshly poured concrete has a high ph; it must also be resistant to high chloride attack from added salts during the life of the structure; and it must not deteriorate or debond with time as this would allow ingress of corrosive fluids to attack the core. Deterioration of the bond has been a problem with the epoxy coatings that have been applied to black rebar in the past.

As already noted, due to the typical length of rebars, it will most often be necessary to mount the caps on the bar ends when the rebar is horizontal and the cap is therefore turned sideways to the position shown in the drawings. Advantageously the sealant, when it is still in the liquid state should be sufficiently viscous to ensure that it does not flow out of the cap under gravity under these circumstances. The viscosity should also be such that, when the skirt of the cap is swaged and the base flattened, the sealant is caused to flow around the bar end rather than escape past the interface between the skirt and the cladding so that any voids tend to be eliminated.

In the present case, the nominal wall thickness of the cap is equal to 0.5 mm. However, the wall thickness can be chosen to suit the thickness of the cladding (that can also vary) as well as cost considerations. By way of example, the thickness of the cladding is typically about 0.5 mm for a 13 mm to 32 mm diameter rebar. For such rebars, a cap of between 0.5 mm to 1.0 mm wall thickness should be suitable for most purposes.

The depth and diameter of the cap is more dependent on the diameter of the rebar. The cap is advantageously loose fitting over the rebar so that it fits easily over the bar end. The free edge of the skirt may be flared as illustrated at 28. Furthermore, allowance should be made for burrs and flashes on the bar ends. However, for rebars up to at least 32 mm in diameter, if the diameter of the skirt is more than a certain amount greater than that of the rebar, the skirt is liable to deform non-uniformly when it is swaged. The cap may thus not be locked tightly on the bar end or may form an imperfect seal. There is thus a practical upper limit to the diameter of the skirt. The following table gives the sizes (in mm) of caps that have been found to be suitable for bars of the diameter shown:

| O/D of Rebar | I/D of Skirt | Depth of Skirt |
|---|---|---|
| 13-16 | 17.2 | 12 |
| 19-22 | 25.1 | 18 |
| 25-32 | 36.3 | 21 |

Clearly, suitable cap sizes can be selected for bars of any size.

Caps of the type described can be swaged on the bar ends by commercially available hydraulically operated machines that are commonly used for swaging end fittings on hydraulic hoses. A suitable such machine is sold under the Hydralok trade mark. Figure 3 shows schematically eight swaging dies 38 arrayed as they are in a swaging machine of this type around the skirt 24 of a cap 20 located at the central axis 40 of the array.

As shown in Figure 4, the machine causes the dies to move radially inwardly towards the axis, deforming the skirt uniformly inwardly and forcing it against the outer face of the cladding on the rebar. Longitudinally extending ribs 42 are formed in the skirt in the process. Excess sealant is able to escape through these ribs. These machines are typically capable of applying up to 1,47×10⁸N (50 tonnes of force). This is sufficient to form an indent in the cladding, serving to lock the cap securely on the bar end.

Machines of this type are inexpensive. An important additional advantage is that they are already used not only in workshops but also on construction sites for joining rebars together. This is achieved by means of a steel sleeve into which the bar ends are inserted end to end, the machine being used to swage the sleeve to each bar end. In workshops, the swaging operation is frequently automated. However, on construction sites, it is more common to find manually operated swaging machines.

Sealing of rebar ends by this method is economical and quick. At the present time, for manually applying end caps to a batch of 120 cut ends of 16 mm diameter rebar, a typical total overall cost per end is of the order of £0.078, being made up of £0,013 for the ss-end cap, £0.019 for the cost of sealant and £0.046 labour cost at £5.50/hr. The labour cost is much reduced if the process is automated. At an average bar length of 4m, the cost of sealing the ends of a tonne of 16 mm rebar would be about £25.

Tests have been carried out on the ends of ss-clad rebars sealed with end caps as described above. In these tests, the capped ends were immersed in an acid solution appropriate for stainless steel for 1-2 hours. This solution comprised 2.5% hydrofluoric and 12% nitric acid. The capped ends were then cyclically immersed an 8% saline solution and then dried over a period of 15 days. These tests were intended to replicate production conditions followed by expected service conditions. The capped ends were then sectioned in order to observe whether the core had been attacked by either the acid or the saline solution.

In some cases the domed ends of the caps were not flattened. Although voids were found in some of these, no attack or rust has been observed on any of the capped ends tested to date.

In an alternative method, a meltable metallic sealant is used instead of the organic sealant described above. Various metallic sealants are suitable, including:
- low temperature melting solders that typically melt at 200-300°C. An example of a suitable corrosion resistant solder is P40 available from Johnson Matthey. This is composed of 96% Sn and 4%Ag;
- silver brazing alloys that melt at 600-800°C. An example is Argobraze 56 or Argobraze 49H available from Johnson Matthey. The melting temperature of Argobraze 56 is 600-711°C. and the specification is 56%Ag, 27%Cu, 14.5%In, 2.5%Ni. Argobraze 56 is specially suited for stainless steel applications in wet conditions;
- high temperature brazing alloys that melt at 800-1050°C. An example of a highly corrosion resistant such alloy is HTN2, also available from Johnson Matthey, and comprising 82.4%Ni, 7%Cr, 3.0%Fe, 3.1%Bo, 4.%Si.

The metallic sealant can be supplied in a cold form (including powder, pellet, wire or disc form) that is suitable for insertion in caps 50 that can be identical to the caps 20. A rebar 56 with a cap 50 mounted thereon is illustrated at the right hand end of Figure 5, the metallic sealant being shown at 52.

When metallic sealant is used, the entire capping and sealing process is advantageously at least partially automated. For this purpose an apparatus, shown schematically at 54 in Figure 6 is used. In this apparatus, a bar 56 is manually or automatically moved to a predetermined position between a pair of hydraulically operated jaws 60 mounted in a transport carriage 62 with the bar end against a locating stop 64. This ensures that the bar end is positioned at the correct axial distance from, and in axial alignment with, a swaging head 66 equipped with a set of swaging dies similar to those shown in Figures 3 and 4. The jaws 60 are then operated to grip the bar and the stop is withdrawn laterally, allowing access to the bar end. A suitable flux is applied to the bar end before a cap 50, with the correct quantity of cold metallic sealant inserted, is manually mounted over the bar end. The transport carriage is then operated to advance the bar in the axial direction so that the bar end, carrying the cap 50, enters the swaging head 66. The swaging dies are operated to swage the skirt of the cap to the cladding of the bar.

The transport head is now again operated to advance the bar 56 further, this time to a position in which the bar end, carrying the swaged cap, enters the coil 72 of a conventional induction heating apparatus. This allows the sealant to be heated to melting point is a matter of seconds. The molten sealant is fluent and migrates to the interface between the skirt and the cladding. At the same time, a dome shaped head 74 is advanced axially towards the bar end. The head 74 bears on the domed base of the cap, flattening it to remove voids 76 in the space between the bar end and the cap.

A seal is formed at the interface when the sealant cools and solidifies. The transport head withdraws the rebar and releases it, thereby allowing the rebar to be manually removed from the apparatus 54. Because the cap is firmly locked on the rebar, it is not necessary to wait for the sealant to solidify.

Many proprietary fluxes are available. Examples are Tenacity 5 and Mattiflux 100 available from Johnson Matthey . Alternatively, ammonium chloride either alone or mixed with aluminium, both in powder form, may be used as fluxes. An advantage of the latter is a reduced possibility of the occurrence of inclusions produced by the flux when it melts.

Using a metallic sealant is likely to be more expensive and more difficult to apply in the field than an organic sealant.

Only in powder form is the raw metallic sealant to some extent fluent before it is heated. Even in powder form, the cold sealant does not flow as readily as liquid sealant. Consequently, voids 76 are to be expected after the skirt is swaged. However, provided that the end face of the bar is reasonably square, such voids are removed when the domed end of the cap is flattened as described above and illustrated at the left hand end of the rebar in Figure 5. If the end face is ragged or not sufficiently square, it may be necessary to increase the amount of raw sealant that is inserted in the cap and, as a consequence, to provide a cap with increased depth.

If a cap with metallic sealant is applied to the cut end of a rebar on site, the cap can be swaged by a hand operated machine as described above, and the sealant heated to melting point by an oxy-acetylene or other suitable gas heating equipment. Such equipment is readily available and, in any case, is used on nearly all construction sites. As before, the domed end of the cap can be flattened by striking it with a hammer.

Before being fitted, the metallic cap is a loose fit over the end of the rebar.

The methods of sealing the bar ends have various advantages in addition to those mentioned:
- They are inexpensive. A few pence cost per bar end translates into a considerable cost per tonne and could edge the cost of clad rebar towards that of solid ss-rebar. Typically for 4m lengths of 16mm rebar there are 320 ends per tonne.
- The caps are quick and simple to apply. In a production situation the process is easy to automate. On site, the process can be carried out by non-skilled personnel.
- The caps cannot be easily damaged or removed. This is so whether due to handling during transportation or on site, during fitting and installation in the structure; or during casting and vibrating concrete.
- It is expected that the end seals will have the same useful life as ss-clad rebar.

## Claims

1. A method of scaling a cut end [13] of an elongate product [10, 56] comprising a core [12] of corrosion susceptible metal and a cladding [14] of corrosion resistant metal bonded to an axially extending outer face of the core, the method being **CHARACTERISED IN** including the steps of providing a capping element [20, 50] that is of corrosion resistant metal and that is shaped so that the capping element can be mounted on the cut end of the product with an exposed portion [18] of the core enclosed by the capping element and a skirt [24] of the capping element overlying a portion of the cladding adjacent the exposed portion of the core, and causing a seal to be present between the skirt and the cladding by steps that include inserting sealant [26, 52] in the capping element and crimping or swaging the skirt so that it is in sealing contact with the cladding, any space between the cut end and the capping element and between the skirt and the cladding being filled by sealant.

2. A method according to claim 1, **CHARACTERISED IN THAT** the capping element is deformed [22"] after it is mounted over the cut end to cause the volume of any space enclosed by the capping element to be reduced.

3. A method according to claim 1, **CHARACTERISED IN THAT** sealant [52] in a non-liquid state is present in the capping element when the capping element [50] is mounted over the cut end, the seal being created by steps that include causing the sealant to become liquid so that it flows between the skirt and the cladding.

4. A method according to claim 3, **CHARACTERISED IN** including the steps of applying heat to cause the sealant to melt so that it flows between the skirt and the cladding, and subsequently allowing the sealant to resolidify.

5. A method according to claim 4, **CHARACTERISED IN THAT** the sealant is metallic.

6. A method according to claim 5, **CHARACTERISED IN THAT** the heat is applied by an induction heating apparatus [72].

7. A method according to any one of claims 1 to 6, in which the core is of engineering steel and the cladding is of stainless steel.

8. A method according to any one of claims 1 to 7, in which the capping element is of corrosion resistant metal.

9. A method according to claim 8 in which the capping clement is of stainless steel.

## Patentansprüche

1. Ein Verfahren des Abdichtens eines abgeschnittenen Endes (13) eines länglichen Erzeugnisses (10, 56), das einen Kern (12) korrosionsanfälligen Metalls und eine Verkleidung (14) korrosionsbeständigen Metalls verbunden mit einer sich axial erstreckenden äußeren Seite der Kerns aufweist, wobei das Verfahren
**DADURCH GEKENNZEICHNET ist, daß** es die Schritte aufweist des Lieferns eines abdeckenden Elementes (20, 50), das aus korrosionsfestem Metall ist und das so geformt ist, daß das abdeckende Element an dem abgeschnittenen Ende des Erzeugnisses angebracht werden kann, wobei ein freiliegender Abschnitt (18) des Kerns durch das abdeckende Element eingeschlossen wird und ein Randgebiet (24) des abdeckenden Elementes einen Bereich der Verkleidung benachbart dem freiliegendem Bereich des Kerns überlagert, und Veranlassen, daß eine Dichtung zwischen dem Randgebiet und der Verkleidung vorhanden ist, durch Schritte, die aufweisen das Einsetzen eines Dichtmittels (26, 52) in dem abdeckenden Element und Crimpen oder Stauchen des Randgebietes so, daß es in dichtender Berührung mit der Verkleidung ist, wobei jeglicher Raum zwischen dem abgeschnittenen Ende und dem abdeckenden Element und zwischen dem Randgebiet und der Verkleidung durch Dichtmittel gefüllt ist.

2. Ein Verfahren nach Anspruch 1, **DADURCH GEKENNZEICHNET, DASS** das abdeckende Element verformt (22") wird, nachdem es über dem geschnittenen Ende angebracht ist, um zu veranlassen, daß das Volumen jeglichen Raumes, der durch das abdeckende Element umschlossen wird, vermindert wird.

3. Ein Verfahren nach Anspruch 1, **DADURCH GEKENNZEICHNET, DASS** Dichtmittel (52) in einem nichtflüssigen Zustand in dem abdeckenden Element vorhanden ist, wenn das abdeckende Element (50) über dem abgeschnittenen Ende angebracht wird, wobei die Dichtung durch Schritte erzeugt wird, die aufweisen, das Dichtmittel zu veranlassen flüssig zu werden, so daß es zwischen das Randgebiet und die Verkleidung läuft.

4. Ein Verfahren nach Anspruch 3, **DADURCH GEKENNZEICHNET, daß** es die Schritte des Anwendens von Hitze, um das Dichtmittel zu veranlassen zu schmelzen, so daß es zwischen das Randgebiet und die Verkleidung läuft, und nachfolgend dem Dichtmittel zu erlauben sich wieder zu verfestigen, aufweist.

5. Ein Verfahren nach Anspruch 4, **DADURCH GEKENNZEICHNET, DASS** das Dichtmittel metallisch ist.

6. Ein Verfahren nach Anspruch 5, **DADURCH GEKENNZEICHNET, DASS** die Hitze durch ein Induktionsheizgerät (72) angelegt wird.

7. Ein Verfahren nach irgendeinem der Ansprüche 1-6, in dem der Kern aus Maschinenbaustahl und die Verkleidung aus rostfreiem Stahl ist.

8. Ein Verfahren nach irgendeinem der Ansprüche 1 - 7, in dem das abdeckende Element aus korrosionsbeständigem Material ist.

9. Ein Verfahren nach Anspruch 8, in dem das abdeckende Element aus rostfreiem Stahl ist.

## Revendications

1. Procédé de scellage d'une extrémité coupée [13] d'un produit allongé [10, 56] comprenant une âme [12] de métal sujet à la corrosion et un gainage [14] de métal résistant à la corrosion lié à une face externe de l'âme s'étendant axialement, le procédé étant **caractérisé en ce qu'**il comprend les étapes consistant à mettre en oeuvre un élément coiffant [20, 50] qui est en métal résistant à la corrosion et qui est façonné de sorte que l'élément coiffant puisse être monté sur l'extrémité coupée du produit avec une partie exposée [18] de l'âme enserrée par l'élément coiffant et une jupe [24] de l'élément coiffant recouvrant une partie du gainage adjacent à la partie exposée de l'âme, et à amener la présence d'un joint étanche entre la jupe et le gainage par des étapes qui comprennent l'insertion de matériau d'étanchéité [26, 52] dans l'élément coiffant et le sertissage ou le refoulement de la jupe pour qu'elle soit en contact d'étanchéité avec le gainage, tout espace entre l'extrémité coupée et l'élément coiffant et entre la jupe et le gainage étant rempli de matériau d'étanchéité.

2. Procédé selon la revendication 1, **caractérisé en ce que** l'élément coiffant est déformé [22"] après avoir été monté sur l'extrémité coupée pour entraîner la réduction d'un espace quelconque enserré par l'élément coiffant.

3. Procédé selon la revendication 1, **caractérisé en ce que** le matériau d'étanchéité [52] à l'état non liquide est présent dans l'élément coiffant lorsque l'élément coiffant [50] est monté sur l'extrémité coupée, le joint étanche étant créé par des étapes consistant à faire en sorte que le matériau d'étanchéité devienne liquide pour qu'il s'insinue entre la jupe et le gainage.

4. Procédé selon la revendication 3, **caractérisé en ce qu'**il comprend les étapes consistant à appliquer de la chaleur pour amener le matériau d'étanchéité à fondre et à s'insinuer entre la jupe et le gainage et à laisser ensuite le matériau d'étanchéité se resolidifier.

5. Procédé selon la revendication 4, **caractérisé en ce que** matériau d'étanchéité est métallique.

6. Procédé selon là revendication 5, **caractérisé en ce que** la chaleur est appliquée par un appareil de chauffage par induction [72].

7. Procédé selon l'une quelconque des revendications 1 à 6, dans lequel l'âme est en acier pour constructions mécaniques et le gainage est en acier inoxydable.

8. Procédé selon l'une quelconque des revendications 1 à 7, dans lequel l'élément coiffant est en métal résistant à la corrosion.

9. Procédé selon la revendication 8, dans lequel l'élément coiffant est en acier inoxydable.
